

# UNITED STATES PATENT OFFICE.

ROBERT W. CORNELISON, OF SOMERVILLE, NEW JERSEY, ASSIGNOR TO THE COTT-A-LAP COMPANY, OF SOMERVILLE, NEW JERSEY, A CORPORATION OF NEW JERSEY.

## CALCIMINE AND PROCESS OF MAKING SAME.

1,244,033.

Specification of Letters Patent.

Patented Oct. 23, 1917.

No Drawing.

Application filed March 27, 1914. Serial No. 827,601.

*To all whom it may concern:*

Be it known that I, ROBERT W. CORNELISON, a citizen of the United States, and a resident of Somerville, in the county of 5 Somerset and State of New Jersey, have invented certain new and useful Improvements in Calcimines and Process of Making Same, of which the following is a specification.

10 My invention relates to the production of colored calcimines and has for its object to simplify considerably the present procedure, to reduce in a very large measure the amount of different materials which a jobber, dealer, 15 or decorator is required to keep in stock in order to supply the demand for different colors (hues) or tints, and to enable the user to produce readily, from a comparatively small number of ingredients kept in small 20 quantities, a large number of different hues and tints, with a certainty that the exact tint or hue desired will be obtained in each case. All the ingredients of my calcimine are kept in dry, solid form, which also 25 makes it easy to put them in containers of different characters, as will be set forth more fully hereinafter.

Heretofore dry prepared calcimines have generally been supplied to the trade and to 30 the user ready mixed, such calcimines consisting essentially of one or more main body substances mixed with adhesive material forming the necessary binder. The pigments most commonly used are clay and 35 whiting, and when desired, tints are produced by incorporating with the mixture, ochre, red oxid, or other suitable coloring matter. The binder is usually glue, or casein with the necessary alkaline substance for 40 solution. These substances are all suitably powdered by grinding, either before, or during, or after the mixing, and the resulting white or tinted calcimine is put up in suitable packages. The manufacturer will supply 45 the dealer with as many different tints and hues, put up in separate packages, as the customers may be expected to call for. Of course, some tints will be more in demand than others, but should there be a 50 sudden demand for some tint not ordinarily kept in stock, or an unusually large demand for some tint of which only a limited supply is on hand, the dealer will not be able to satisfy his customers at once; in fact, in

order to be prepared for a shifting in the 55 customers' demands, the dealer will be compelled to keep a much larger stock than the actual sales would require, thus increasing the capital and interest charges.

According to my invention, I employ a 60 single calcimine body, which the dealer would keep in stock separately, and a limited number (say, three different kinds only) of coloring bodies, made in accurately pre-determined quantities, and I also provide 65 a chart showing a large number of hues and tints, together with the exact number of color units (of one or more kinds) which must be combined with one body unit to produce the several hues and tints shown 70 on the chart. The dealer would therefore have to keep in stock, only a number of body units according to the needs of his trade, a number of say yellow color units, a number of red color units, and a number of blue 75 color units. All the body units would be of the same weight, and all units of the same color would be of the same weight; preferably, the units of all colors would be of the same weight, and in any event, the 80 weight of the color units would be small relatively to the weight of the body units. In the preferred form of my invention, the calcimine body would contain a color-lake-producing material, while the color units 85 would consist of lake-forming coloring matters. I am thus enabled to employ a class of coloring matters different from those used heretofore, namely, soluble dyes, and thereby can attain a very much higher degree of 90 concentration of the color units (and therefore reduced bulk) as well as a more thorough distribution, and other advantages which will be pointed out hereinafter.

The calcimine body employed according 95 to this preferred form of my invention, comprises, besides the color-lake-producing material, a main portion consisting of a suitable binder and of the above-mentioned main body substances which form the chief 100 constituents of the finished product. For example, the calcimine body may consist of color-lake-producing material and of a mixture of ground glue with whiting, china clay, or other similar substance or substances. These latter substances I shall herein call the main body substances. Usually 105 they are white or nearly so, and inexpen-

sive; they should be in a state of fine subdivision. By the term "color-lake-producing material" I designate a substance or substances which will combine, or some part 5 or constituent of which will combine, with a suitable soluble dye to form insoluble colored pigments (or a pigment of this character) of the class usually called color lakes. As example of color-lake-producing mate- 10 rials, as I have just defined them, I would mention barium chlorid, alumina, or other basic matter similar thereto. It will be obvious that I may use alum as a source of aluminum, or I may employ some other salt 15 of aluminum, chromium, iron, or other metal. Some dyes will precipitate and form color lakes with basic phosphates, silicates, and the like.

The color units, in the preferred form of 20 my invention, are lake-forming coloring matter's, as I have stated above. By this term I designate a dye which has the property of combining with the material which I have termed "color-lake-producing mate- 25 rial" as defined above, to form an insoluble pigment. For example, many of the commercial azo dyes are sodium salts of color acids and are soluble in water while the corresponding barium salts are insoluble or 30 nearly so. When a solution of the sodium salt of the azo color comes in contact with a solution of barium chlorid, there occurs a double decomposition resulting in the formation of sodium chlorid and the barium salt 35 of the azo compound, *i. e.*, a color lake. The formation of color lakes such as mentioned in connection with my invention, usually involves chemical action and takes place only in the presence of water.

40 It is a well-known fact that a soluble dye remaining in this condition is not a suitable coloring material for a calcimine. By my improved process I am enabled to produce in and throughout the calcimine body, *in 45 situ*, so to speak, in a state of very fine subdivision, a colored constituent, namely, a colored pigment or lake which at once imparts its tint to the whole mixture. It is well understood that this color-lake has not 50 previously existed as such in any of the constituents of my improved calcimine, although of course, the ingredients required for the production of such color lake were present in the constituents of my calcimine.

55 An example of my invention is as follows:—For the new calcimine body I make a mixture of

500 grams of whiting,  
405 grams of china clay,  
45 grams of powdered glue,  
50 grams of sulfate of aluminum,

making 1000 grams in all. The whole being finely powdered and thoroughly mixed, is 60 put up in suitable containers, such as cans,

in exactly measured amounts, for instance of 500 grams or 1000 grams each. This calcimine body is dry and solid, that is to say, it is not paste-like or liquid, although preferably in the powdered condition, so 70 that it will readily mix with water. The bulk or greater portion of this calcimine body is insoluble in water, and will simply become suspended in water when mixed therewith.

75 As suitable lake-forming coloring mat- ters, for use with the above calcimine body, the following may be used, for example:

For yellow, chrysophenin G concentrated (Bayer).

80 For red, diamin rose B extra (Cassella).

For blue, indigo carmine (Schultz & Jules) (Green's translation, #692).

It will be understood that the above are given as examples only, which I have se- 85 lected chiefly because they are well-known dyes and are typical of dyes which, for the greater part at least, are precipitated by a mixture of aluminum sulfate with an ex- cess of calcium carbonate (whiting). Chry- 90 sophenin G concentrated is very fast to light, but as to blue, there are other sub- stances more suitable in this respect than indigo carmine. Diamin rose B extra is only moderately fast to light. Still in many 95 cases, the particular substances named above will do very well; in some cases, however, I prefer to select dyes which are exceed- ingly fast both to light and to alkalis.

As stated, I may use many other dyes, and 100 for certain purposes there may be others more suitable than the particular ones named, yet with the yellow, red and blue named above I can obtain almost every shade that may be desired. Furthermore, 105 in view of the concentrated condition in which these substances are readily purchas- able, a comparatively small amount of the lake-forming coloring matter is sufficient 110 to produce tints of the depth usually re- quired for calcimine work. The lake-form- ing coloring matters would be sold in accu- 115 rately measured quantities, say of 1 gram, either as loose powder, but preferably in co- herent form, as small blocks or tablets. When used as a loose powder, these sub- 120 stances may be put in paper bags, metal cans, capsules, or other suitable containers. When provided as coherent blocks or tablets (each of a weight equal to the particular unit adopted, which unit of course is much smaller than that of the calcimine body), the lake-forming coloring matters might be wrapped in paper (with a suitable label), or sold in suitable containers, or even with- 125 out any containers, since tablets, even of dif- ferent colors, may be kept in the painter's pocket as he goes to his job, without any danger of getting mixed. If the tablets, for the sake of convenience and as a protec- 130

tion against soiling and crumbling, are put in a container, there is no necessity of providing a separate container for each color, but owing to their coherent nature, tablets 5 of the same or of different colors may be kept in the same container without any danger of their getting mixed. If desired, a suitable designation or mark (such as Blue or B) may be placed on each tablet, for instance by molding such word or mark in the 10 tablet at the time of forming the tablet.

In any event, both the body units and the color units (or units of color-lake forming material) are solid, that is to say, not pasty 15 or liquid. The advantages derived from using the materials or ingredients in this condition are manifold. Less expensive packages or containers can be used, paper bags or envelops being sufficient in many 20 cases, and as stated above, the container may even be dispensed with altogether when the units are made in coherent bodies such as tablets. It will also be obvious that as to shipping, solid dry substances such as are 25 used in my invention, offer material advantages over liquid or paste-like substances, first, in that accompanying freight will be less exposed to damage in case the package containing the calcimine ingredients should 30 be broken so as to allow its contents to come in contact with accompanying goods, and second, the shipping expense is lower on account of the absence of the liquid portion (water), which is readily obtainable any- 35 where. I also avoid all corroding action of contents on container, which in the case of liquid or paste-like ingredients is a frequent source not only of damage to the container, but of contamination of the ingredients re- 40 sulting in delicate tints being thrown off color. I further avoid changes in shade such as may be caused by chemical action between tinted materials and a liquid vehicle, or by the action of tinted materials 45 on each other if allowed to stand for long periods of time in the presence of a liquid. Finally, it is well-known that in mixed paints of a liquid or semi-liquid character, the settling of certain ingredients, and par- 50 ticularly pigments, is liable to form a hard mass at the bottom of the container, so that the paint, if usable at all, can be made serviceable only by much labor in stirring and mixing it to restore the proper homo- 55 geneous condition. All these defects and dangers are avoided by the use of solid, dry ingredients according to my invention.

To recapitulate, in the preferred form of my invention, there would be prepared, and 60 offered for sale by the dealers, only a limited number of different "units", of which four kinds would generally be sufficient for all requirements occurring in practice, viz.: (1) body units, say of 1000 grams each; (2) 65 units of yellow lake-forming coloring mat-

ter; (3) units of red lake-forming coloring matter; and (4) units of blue lake-forming coloring matter. The three kinds of color units named under 2, 3, and 4 would be say of 1 gram each, and preferably in the form 70 of compressed tablets. In addition to these several units, the dealer would keep a chart (copies of which might also be given to prospective users) showing the numerous tints and hues that could be obtained by employing a body unit with one or more color units. The body unit, used alone, would produce a substantially white color. One body unit (say 1000 grams) with one blue color unit (say 1 gram) would produce a very light 80 blue tint; if two blue color units are used with one body unit, a somewhat deeper shade of blue would be obtained, and thus, by increasing the number of blue units per body unit, still deeper shades of blue would 85 be produced. In the corresponding way, lighter or darker red calcimines could be obtained by using one body unit with one or more red units, and similarly, different shades of yellow could be produced. By 90 employing the body unit in conjunction with one or more blue units and one or more yellow units, various shades of green would be obtained. Thus, by using the body unit in conjunction with one or more color units, 95 either of the same color, or of two or three different colors (yellow, red, and blue), a very large number of different tints and hues could be produced. The chart would show not only the different tints and hues obtainable by means of my body unit and color units, but also the exact composition of each hue or tint, for instance indicating that a particular tint required three red units, two 100 blue units, and one yellow unit for each body 105 unit. If the color units are sold in envelops or other containers, it might be convenient to place on the outside of such container a portion of the color chart, that is to say, a partial chart showing only those tints which 110 would result from using units of that particular color (say, red) exclusively in connection with the body unit (that is to say, in this particular case, the different shades of red obtained by using the body unit with one 115 or more red color units). The user could therefore ascertain very readily how to produce any one of the various tints or hues shown on the chart, and it will be obvious that with red, blue, and yellow color units, all tints and hues ordinarily required could 120 be produced, the number of possible combinations being exceedingly large.

The method of using my improved calcimine is as follows: For a small ceiling 1 unit 125 of calcimine body (1 kilogram) is usually sufficient. The workman, therefore, carries one body unit and an assortment of color units. The latter being exceedingly small (say, 1 gram each), the workman could read- 130

ily carry a complete assortment, sufficient for all ordinary purposes, in his vest pocket. Having arrived at the job, the workman would show the color chart to the customer, 5 who would then select the desired color from the chart. By referring to the chart, the workman would ascertain at once how the desired color is to be produced, that is to say how many units of each color he will 10 have to use for one unit package of calcimine body. He then counts out the correct number of tablets, or other forms of color units, and throws them into some water. He also takes a unit of calcimine body and mixes it with 15 slightly less than the requisite amount of water. When both the color units and the body unit are thoroughly disintegrated and mixed with the water, the two liquids are poured together and the mixture stirred thoroughly. Another good way (which I prefer in 20 practice) is to first disintegrate the color units in water and then mix the liquid with the body unit. The amount of water required in each case will be readily ascertained by any 25 man familiar with calcimining. I suggest  $1\frac{1}{2}$  liters of water to 1 kilogram of body unit. The calcimine is applied to the ceiling or other surface, in the usual way.

It will be obvious that each color unit may 30 contain only one lake-forming coloring matter, as in the examples given above, or a mixture of two or more substances of this character, suitable for the production of the desired result. All these substances, however, 35 should be capable of forming insoluble pigments with the color-lake-producing material contained in my calcimine body. (In the particular example of calcimine body given above, the sulfate of aluminum is the color-lake-producing material). Of course, I do 40 not wish to confine myself to the exact formula or ingredients named above for the calcimine body, or to the particular colors or classes of colors indicated. Obviously, I 45 might use quite different materials, for instance the so-called basic colors, and add tannic acid to my calcimine body. Again, there are many dyestuffs which form lakes with salts of lead (for example, naphthol green 50 B.), of copper, and of other metals.

If aluminum sulfate and whiting be used, chemical action begins as soon as the calcimine body comes in contact with water. From aluminum sulfate, calcium carbonate 55 (whiting), and water, there is produced calcium sulfate, aluminum hydroxid, and carbon dioxid. Upon the addition of the color units, aluminum lakes of such colors would be formed.

60 By reason of the high degree of concentration in which lake-forming coloring matter is obtainable commercially, it is not necessary to add more binder (adhesive material) to my calcimine when the color units 65 are added. The comparatively small weight

of color necessary enables the workman to carry a large assortment of colors in his pocket (as stated above), and he may color my calcimine body any shade desired at the time it is applied. It is to be understood 70 that I employ the color-lake-producing material in such proportions as to precipitate the lake-forming coloring matter in sufficient quantity to render insoluble or pigmentize, so to speak, enough of said coloring matter to meet the requirements of the ordinary calcimine. 75

As I have pointed out above, I might use barium chlorid and various other metallic salts as the color-lake-producing matter, 80 but for most work I prefer aluminum sulfate, and calcium carbonate in the form of whiting. I may add other ingredients to the calcimine body, such as china clay, etc. When I employ aluminum sulfate and an 85 equivalent quantity, or an excess of calcium carbonate, it is evident that I do not increase materially the proportion of soluble salts in the resultant mixture. Any excess of aluminum hydroxid and calcium sulfate 90 over and above that necessary for the precipitation of the dyestuff, is valuable as white pigment in addition to that already contained in the calcimine body, for example, china clay. I might also mention 95 that when using comparatively large quantities of aluminum sulfate and calcium carbonate, as I do in my invention, or at least in its preferred form, the carbonic acid generated is decidedly beneficial, inasmuch 100 as it assists in producing a thorough mixture of the calcimine body with water, by breaking up any lumps which might tend to form otherwise. The same result may be obtained by incorporating effervescent 105 material, such as for instance bicarbonate of soda and oxalic acid, either in the body units or in the color units.

Various modifications may be made without departing from the nature of my invention as set forth in the appended claims. 110

I claim as my invention:

1. A prepared calcimine comprising a body containing, in addition to a measured quantity of solid ingredients the bulk of 115 which is insoluble in water, effervescent material which will assist the disintegration of the body when in contact with water, together with color-lake-producing material, and color units containing lake-forming 120 coloring matter complementary to said coloring matter, and effervescent material distributed throughout the color units to assist their disintegration when in contact with water.

2. In the art of preparing a colored calcimine, the step which consists in bringing together a color-lake-producing material, a calcimine body, and lake-forming coloring matter. 125 130

3. A calcimine comprising lake-forming coloring matter, and a calcimine body which contains a color-lake-producing material.
4. In the art of preparing colored calcimine, the improvement which consists in bringing together a lake-forming coloring matter and a calcimine body which contains color-lake-producing material.
5. A calcimine comprising lake-forming coloring matter, and a calcimine body containing dye-precipitating material.
6. A calcimine containing glue and a salt of a metal, together with precipitating material for said salt, and a soluble dye, which dye will form a color lake in and throughout the calcimine with a compound of the said metal, substantially as set forth.
7. The process of precipitating a color lake in and throughout a prepared calcimine containing a suitable binder, which consists in introducing into the calcimine, material which will form an insoluble com-

pound with a soluble dye, and adding a lake-forming dye in the presence of water.

8. The process of coloring a calcimine, which consists in incorporating a precipitant with the calcimine body and then adding a soluble dye which, by the action of said precipitant, will be precipitated in and throughout the said calcimine.

9. The process of coloring a calcimine, which consists in incorporating with the calcimine body, a lake-producing precipitating material, and then adding a soluble dye adapted to form a color lake with said precipitating material.

In testimony whereof, I have signed this specification in the presence of two subscribing witnesses.

ROBERT W. CORNELISON.

Witnesses:

JOHN LOTKA,  
CHARLES A. MATHI.